

## [54] ALKANOLAMINES AS COLD-END ADDITIVES

[75] Inventors: Bruce L. Libutti, Pompton Plains; Francis J. Oschell, Stanhope, both of N.J.

[73] Assignee: **Betz Laboratories, Inc.**, Trevose, Pa.

[\*] Notice: The portion of the term of this patent subsequent to Jan. 16, 1996, has been disclaimed.

[21] Appl. No.: 955,829

[22] Filed: Oct. 30, 1978

## Related U.S. Application Data

[63] Continuation-in-part of Ser. No. 833,797, Sep. 16, 1977, Pat. No. 4,134,728, which is a continuation of Ser. No. 713,727, Aug. 12, 1976, abandoned.

[51] Int. Cl.<sup>2</sup> ..... C23F 11/00; C23F 11/02

[52] U.S. Cl. ..... 422/9; 110/343; 110/345; 252/392; 423/242; 423/243; 423/244

[58] Field of Search ..... 422/9; 423/242, 243, 423/244; 110/343, 345; 252/389 R, 392

## [56] References Cited

## U.S. PATENT DOCUMENTS

|           |         |                 |           |
|-----------|---------|-----------------|-----------|
| 2,106,446 | 1/1938  | Baehr et al.    | 423/243 X |
| 2,155,853 | 4/1939  | Anthony         | 423/243 X |
| 2,972,861 | 2/1961  | Davies          | 422/9 X   |
| 3,343,908 | 9/1967  | Wickert         | 423/244   |
| 3,547,583 | 12/1970 | Wilson          | 423/242   |
| 3,709,977 | 1/1973  | Villiers-Fisher | 423/244   |
| 3,720,754 | 3/1973  | Wilson          | 423/244   |
| 3,809,745 | 5/1974  | Wilson          | 423/244   |

|           |         |                 |           |
|-----------|---------|-----------------|-----------|
| 3,856,921 | 12/1974 | Shrier et al.   | 423/243 X |
| 3,873,673 | 3/1975  | Teague et al.   | 423/243   |
| 3,886,261 | 5/1975  | Libutti         | 423/244   |
| 3,904,735 | 9/1975  | Atwood et al.   | 423/243   |
| 3,932,588 | 1/1976  | Libutti et al.  | 423/244   |
| 3,961,018 | 6/1976  | Williamson      | 423/243 X |
| 3,962,404 | 6/1976  | Giammano et al. | 423/243 X |

## FOREIGN PATENT DOCUMENTS

|         |        |                |         |
|---------|--------|----------------|---------|
| 872984  | 7/1961 | United Kingdom | 423/244 |
| 1305750 | 2/1973 | United Kingdom | 423/244 |

## OTHER PUBLICATIONS

Bienstock et al., "Process Development in Removing Sulfur Dioxide from Hot Flue Gases", Report No. 5735, Bureau of Mines (pp. 8-17).

Gundry et al., "The Use of Ammonia for Reducing Air-Heater Corrosion at Bankside Generating Station, C.E.G.B.", vol. 36, *Combustion*; 10/64; pp. 39-47.

Primary Examiner—Barry S. Richman  
Attorney, Agent, or Firm—Alexander D. Ricci; Steven H. Markowitz

[57]

## ABSTRACT

A method of reducing the amount of sulfur trioxide condensation on, and therefore the amount of sulfuric acid corrosion of, metal parts at the cold-end of a combustion system and in contact with combustion gases derived from the combustion of sulfur containing fuel, said method comprising adding to the combustion gases an effective amount for the purpose of an aliphatic, water-soluble alkanolamine additive.

13 Claims, No Drawings

## ALKANOLAMINES AS COLD-END ADDITIVES

This application is a continuation-in-part of Ser. No. 833,797, filed on Sept. 16, 1977, and now U.S. Pat. No. 4,134,728 issued Jan. 16, 1979, which is a continuation of Ser. No. 713,727, filed Aug. 12, 1976 and now abandoned.

## DISCLOSURE OF THE INVENTION

As is well known to boiler operators, sulfur-containing fuels present problems not only from a pollutional point of view, i.e., acid smut, but also with respect to the life and operability of metallic equipment and parts which are in contact with the flue gases containing the sulfur by-products of combustion.

Upon combustion, the sulfur in the fuel is converted to sulfur dioxide and sulfur trioxide. When sulfur trioxide reaches its dew temperature, it reacts with moisture in the flue gas to produce the very corrosive sulfuric acid. The gases themselves are troublesome as air pollutants, while the acid formed is damaging from corrosion aspects.

As can be appreciated, the greater the sulfur content of the fuel, the more the effects are harmful. This is particularly the case in industrial and utility operations where low grade oils are used for combustion purposes.

Although many additives have been utilized for the purpose of conditioning flue gases, few additives have found overall success. The reason for the relatively little success in this area is felt to be the peculiarities found in the different combustion systems and boiler designs. The gas dynamics and the loads produced sometimes make chemical treatments for the most part impractical, therefore requiring a combination of mechanical and chemical treatment.

The basic area to which the present invention is directed is often referred to in the industry as the "cold-end" of a boiler operation. This area is generalized as being the path in the boiler system that the combustion gases follow after the gases have, in fact, performed their service of heating water, producing steam and/or superheating steam.

In the larger boiler systems, the last stages through which the hot combustion gases flow include the economizer, the air heater, the collection equipment or the electrostatic precipitator, and then the stack through which the gases are discharged.

In three articles, a first entitled "The Selection and Use of Additives in Oil-fired Boilers," by W. D. Jarvis and appearing in the November, 1958, issue of the *Journal of the Institute of Fuel*; a second entitled "The Use of Ammonia for Reducing Air-heater Corrosion at Bankside Generating Station, C.E.G.B.," by J. T. S. Gundry, B. Lees, L. K. Rendle, and E. J. Wicks and appearing in the October, 1964, issue of *Combustion*; and a third entitled "The Use of Heterocyclic Tertiary Amines for the Control of Corrosion Caused by Flue Gases," by E. Brett Davies and B. J. Alexander and appearing in the April, 1960, issue of the *Journal of the Institute of Fuel*; the use of heterocyclic tertiary amines, obtained from the distillation of crude coal tar, as boiler cold-end additives is disclosed. Besides disclosing that heterocyclic tertiary amines inhibit boiler cold-end corrosion, the articles also point out that the use of these chemicals causes black carbonaceous deposits on cold-end surfaces, which deposits can become pasty and have a

pronounced smell, apparently due to their derivation from coal tar.

The present invention is drawn to the present inventor's discovery of aliphatic, water-soluble alkanolamines as cold-end additives.

It was determined that if such an alkanolamine (or mixture of alkanolamines) is fed, preferably in droplet form to the moving combustion gases upstream of the cold-end surfaces to be treated and at a point where the gases are undergoing turbulence, the chemical will travel along with the gases as vapor and/or liquid droplets and deposit on the downstream cold-end surfaces. The deposition of the alkanolamine on the cold-end surfaces results from the transition of the gas flow from a zone of relative turbulence to a zone where the turbulence subsides and/or from the lowering of the temperature of combustion gases below the dew point of the chemical. In addition, droplets will impact on the surfaces. It is understood that any reference to an alkanolamine is intended to include mixtures of such compounds.

The liquid additive can be fed as an aqueous solution, and, as noted above, to ensure effective results, the additive is preferably fed in droplet form to the gases and in a zone of turbulence upstream of the surfaces to be treated. There are numerous methods available to the artisan for feeding the additive in droplet form, which methods are deemed well within the skill of the art. For example, liquid atomizer nozzles could be utilized for the purpose. The present inventor obtained satisfactory results using a sonic feed nozzle to produce a mist of the additive solution even though additive deposits formed on the nozzle. The use of a pressure atomizing nozzle system with in-line dilution and water purging should resolve any problems related to the formation of deposits on the nozzle. The size range of the liquid droplets is preferably small enough to ensure that the additive which does not evaporate, but, instead, is present in the combustion gases in liquid droplet form, will be carried along with the combustion gases so as to be deposited on the surfaces to be treated. Based upon the present inventor's prior experience in this area, the size of the droplets could be as large as about 360 microns with the preferred maximum size being about 260 microns. The amount of the alkanolamine added is a function of the sulfur content of the fuel, and, more specifically, the SO<sub>3</sub> (sulfur trioxide) produced upon combustion. On an actives basis, as little as about 0.1 pound of alkanolamine per pound of SO<sub>3</sub> generated could be used. The preferred minimum is about 0.25 pound of alkanolamine per pound of SO<sub>3</sub>. Based on economic considerations, the amount of active additive fed could be as high as about 1.0 pound per pound of SO<sub>3</sub> while about 0.33 pound of alkanolamine per pound of SO<sub>3</sub> represents the preferred maximum. It should be understood, however, that the demands of a particular cold-end problem could call for higher amounts of additive, up to about 2 pounds per pound of SO<sub>3</sub> generated.

The temperature of the combustion gases at the time of addition is from about 250° F. to about 675° F., preferably from about 350° F. to about 650° F.

In order to assess the efficacy of the inventive materials, various tests were conducted on industrial boiler systems which were fired by fuel oil containing about 2.2 percent sulfur. The abilities of the inventive additive to coat surfaces and to reduce acid deposition, corrosion, and fouling were evaluated. Acid deposition rates at various surface temperatures were determined by

titrating washings from a standard air-cooled CERL probe. The nature of the surface coating was determined by visual inspection of the probe. The washings were also analyzed for total iron and total solids content to obtain indications of corrosion rates and fouling tendencies, respectively. Using a Land meter, the rate of acid build-up (RBU) was determined.

The material tested was commercially available N-aminoethyl ethanolamine (Naeaa) which was obtained from Union Carbide. The additive was mixed with 10 water and a commercially available sodium salt of EDTA (as a stabilizer) to form an aqueous solution

while, in the confirming tests, the probe was exposed for the time periods indicated.

TABLE 1A

| Additive | Feedrate (pph) | Steam Load (pph $\times 10^3$ ) | % O <sub>2</sub> | Acid Deposition 220° F. |
|----------|----------------|---------------------------------|------------------|-------------------------|
| None     | —              | 50                              | 2.75             | 10.5                    |
| None     | —              | 56                              | 3.0              | 13.0                    |
| None     | —              | 56                              | 2.9              | 14.0                    |
| Naeaa    | 1.2            | 53                              | 3.7              | 8.0                     |
| Naeaa    | 3.4            | 50                              | 3.8              | 5.5                     |
| Naeaa    | 3.4            | 50                              | 3.8              | 4.0                     |

TABLE 1B

| Additive | Exposure Time (hrs) | Feedrate (pph) | Steam Load (pph $\times 10^3$ ) | % O <sub>2</sub> | Acid Deposition |         |
|----------|---------------------|----------------|---------------------------------|------------------|-----------------|---------|
|          |                     |                |                                 |                  | 250° F.         | 230° F. |
| None     | 0.5                 | —              | 100                             | 2.5-3.0          | 28              | 38      |
| None     | 0.5                 | —              | 100                             | 2.5-3.0          | 28              | 38      |
| None     | 0.5                 | —              | 114                             | 2.5-3.0          | 32              | 46      |
| None     | 3.0                 | —              | 104                             | 2.5-3.0          | 72              | 108     |
| Naeaa    | 0.5                 | 2.8            | 100                             | 2.5              | 9               | 12      |
| Naeaa    | 0.5                 | 1.2            | 100                             | 2.5              | 12              | 20      |
| Naeaa    | 3.0                 | 3.05           | 104                             | 2.5-3.0          | 64              | 76      |
| Naeaa    | 3.0                 | 3.1            | 104                             | 2.5-3.0          | 32              | 34      |
| Naeaa    | 0.5                 | 4.1            | 114                             | 2.5-3.0          | 10              | 10      |

comprising 49.9% water, 50% Naeaa and 0.1% stabilizer. The additive solution was fed to the combustion gases in a duct at the cold-end of the systems, using an atomizer nozzle located in the duct.

In a first series of tests, which will hereinafter be referred to as the preliminary tests, the combustion gases contained about 18 parts of sulfur trioxide per million parts of combustion gases on a volume basis.

In a second series of tests, which will hereinafter be referred to as the confirming tests, the combustion gases contained about 55 parts of sulfur trioxide per million parts of combustion gases on a volume basis.

#### EXAMPLE 1

As already noted, the effects of the inventive additive on acid deposition rates at various surface temperatures were determined by titrating washings from a probe similar to a standard British Central Electricity Research Laboratories (CERL) acid deposition probe. The construction and operation of this probe are well known in the art as evidenced by an article entitled "An Air-cooled Probe for Measuring Acid Deposition in Boiler Flue Gases" by P. A. Alexander, R. S. Fielder, P. J. Jackson, and E. Raask, page 31, Volume 38, *Journal of the Institute of Fuel*; which is hereby incorporated by reference to indicate the state of the art. Washings from the probe were titrated for sulfuric acid with sodium hydroxide.

The results of these tests are reported in Tables 1A and 1B below in terms of acid deposition rate expressed as milliliters of 0.01 N NaOH needed to titrate one fourth of the amount of acid which deposited on 18.8 square inches (in<sup>2</sup>) to the phenolphthalein endpoint. The feedrates reported are expressed as pounds of active additive per hour, and the steam loads reported are also expressed as pounds per hour. The % O<sub>2</sub> reported is the oxygen content of the combustion gases on a % volume basis. Table 1A contains the results of the preliminary tests, and Table 1B contains the results of the confirming tests. In the preliminary tests, the acid deposition rates at 220° F. were determined, while in the confirming tests the determinations were for acid deposition at 230° F. and 250° F. In the preliminary tests, the probe was exposed to the combustion gases for thirty minutes;

From the results reported in Tables 1A and 1B it can be seen that the rate of acid deposition on the probe was reduced when the N-aminoethyl ethanolamine was added to the combustion gases. This reduction in the acid deposition rate reflects the efficacy of the additive as a neutralizing agent.

#### EXAMPLE 2

In a second series of tests, the efficacy of the inventive additive with respect to lowering the apparent acid dew point in the cold-end of the boiler systems was evaluated. Using a commercially available Land dew point meter, the condensation of a conducting film of sulfuric acid on a controlled temperature probe tip was detected by the onset of the flow of electric current between electrodes embedded in the tip. This permitted the determination of the apparent acid dew point, and comparative rates of acid build-up directly on probe surfaces were obtainable from the rate of increase in current with time at any tip temperature. The results of these tests are reported in Tables 2A and 2B below. The feedrate of active additive and the boiler steam load are both expressed as pounds per hour, the apparent dew points are expressed as degrees Farenheit (°F.) and the rates of acid build-up (RBU) are expressed as microamperes per minute ( $\mu$ amp min<sup>-1</sup>). Table 2A contains the results of the preliminary tests, and Table 2B contains the results of the confirming tests. The rate of acid build-up was determined only for a portion of the tests as indicated in the Tables and was determined at a probe surface temperature of 230° F. for both tests. A reported range for a RBU reading indicates that the RBU changed during the test. The apparent acid dew point is defined as that temperature at which an acid film contacts a surface, at the cold-end in this instance.

TABLE 2A

| Additive | Feedrate (pph) | Steam Load (pph $\times 10^3$ ) | % O <sub>2</sub> | Dew Point (°F.) | RBU |
|----------|----------------|---------------------------------|------------------|-----------------|-----|
| None     | —              | 50                              | 3.75             | 273             | 110 |
| None     | —              | 50                              | 3.75             | 278             | —   |
| None     | —              | 50                              | 3.75             | 277             | —   |
| None     | —              | 53                              | 4.1              | 270             | 140 |

TABLE 2A-continued

| Additive | Feedrate<br>(pph) | Steam Load<br>(pph $\times 10^3$ ) | % O <sub>2</sub> | Dew Point<br>(°F.) | RBU |
|----------|-------------------|------------------------------------|------------------|--------------------|-----|
| None     | —                 | 53                                 | 4.1              | 270                | —   |
| Naeaa    | 3.4               | 50                                 | 3.7              | 122                | 0   |
| Naeaa    | 3.4               | 50                                 | 3.7              | 121                | —   |
| Naeaa    | 1.2               | 53                                 | 4.1              | 265                | 27  |
| Naeaa    | 1.2               | 53                                 | 4.1              | 266                | —   |
| Naeaa    | 2.4               | 53                                 | 3.9              | 195                | 3   |
| Naeaa    | 2.4               | 53                                 | 3.9              | 191                | —   |

TABLE 2B

| Additive | Feedrate<br>(pph) | Steam Load<br>(pph $\times 10^3$ ) | % O <sub>2</sub> | Dew Point<br>(°F.) | RBU     |
|----------|-------------------|------------------------------------|------------------|--------------------|---------|
| None     | —                 | 100                                | 2.5-3.0          | 300                | —       |
| None     | —                 | 100                                | 2.5-3.0          | —                  | 225     |
| None     | —                 | 100                                | 2.5-3.0          | 292                | 225     |
| None     | —                 | 100                                | 2.5-3.0          | 304                | 150     |
| None     | —                 | 100                                | 2.5-3.0          | 294                | 250     |
| None     | —                 | 104                                | 2.5-3.0          | —                  | 200-300 |
| None     | —                 | 104                                | 2.5-3.0          | 295                | —       |
| None     | —                 | 104                                | 2.5-3.0          | 300                | 200     |
| None     | —                 | 114                                | 2.5-3.2          | 293                | 400     |
| None     | —                 | 124                                | 2.5-3.0          | 296                | —       |
| None     | —                 | 124                                | 2.5-3.0          | 300                | —       |
| Naeaa    | 1.3               | 100                                | 2.7              | 280                | —       |
| Naeaa    | 3.1               | 101                                | 2.5-2.7          | —                  | 12      |
| Naeaa    | 4.5               | 104                                | 2.5-3.0          | 140                | —       |
| Naeaa    | 3.8               | 104                                | 2.5-3.0          | 155                | —       |
| Naeaa    | 3.5               | 104                                | 2.5-3.0          | 260                | —       |
| Naeaa    | 3.1               | 104                                | 2.5-3.0          | 180                | 8       |
| Naeaa    | 4.5               | 114                                | 2.5-3.0          | 150                | —       |
| Naeaa    | 2.1               | 114                                | 2.5-3.0          | 290                | —       |
| Naeaa    | 2.5               | 114                                | 2.5-3.0          | 200                | —       |
| None     | —                 | 116                                | 2.5-3.0          | 300                | 420-560 |
| Naeaa    | 1.3               | 116                                | 2.5-3.0          | 300                | 300-500 |

From Tables 2A and 2B it can be seen that the additive is efficacious both with respect to lowering the apparent acid dew point in the cold-end and with respect to decreasing the rate of acid build-up directly on surfaces in the cold-end. By lowering the apparent acid dew point, the chance of the acid condensing in the cold-end of the boiler system at a given temperature is decreased. Furthermore, by lowering the apparent acid dew point in the cold-end, the combustion gas temperature can be lowered, resulting in an increase in boiler efficiency without a corresponding increase in corrosion of surfaces at the cold-end.

#### EXAMPLE 3

Using a portion of the washings obtained from the CERL probe described in Example 1, above, the efficacy of the inventive additive with respect to protecting cold-end surfaces against corrosion was evaluated. Since the iron (Fe) content of the washings indicated the amount of corrosion of the test surfaces exposed to the combustion gases, comparisons of the iron content of the washings provided a method of evaluating the efficacy of the inventive material. The results of these comparative tests are reported below in Tables 3A and 3B, with Table 3A containing the results of the preliminary tests and Table 3B containing the results of the confirming tests. In the preliminary tests, the probe was exposed to the combustion gases for 0.5 hour, and in the confirming tests the probe was exposed for the periods as indicated in Table 3B. The steam loads and active

additive are expressed as pounds per hour (pph), the oxygen content of the combustion gases as percent oxygen (% O<sub>2</sub>) by volume, and the iron content as parts of iron per million parts of washing liquid at the probe temperatures indicated.

TABLE 3A

| Additive | Feedrate<br>(pph) | Steam Load<br>(pph $\times 10^3$ ) | % O <sub>2</sub> | Iron (ppm) |         |
|----------|-------------------|------------------------------------|------------------|------------|---------|
|          |                   |                                    |                  | 230° F.    | 250° F. |
| None     | —                 | 50                                 | 3.7              | 3          | 2       |
| Naeaa    | 3.4               | 50                                 | 3.8              | 2          | 3       |
| Naeaa    | 1.2               | 53                                 | 4.1              | 8          | 6       |

TABLE 3B

| Additive | Expo-<br>sure<br>(hours) | Feed-<br>rate<br>(pph) | Steam Load<br>(pph $\times 10^3$ ) | % O <sub>2</sub> | Iron (ppm) |         |
|----------|--------------------------|------------------------|------------------------------------|------------------|------------|---------|
|          |                          |                        |                                    |                  | 230° F.    | 250° F. |
| None     | 0.5                      | —                      | 100                                | 2.5-3.0          | 70         | 55      |
| None     | 0.5                      | —                      | 100                                | 2.5              | 60         | 25      |
| None     | 3                        | —                      | 104                                | 2.5-3.0          | 130        | 70      |
| None     | 6                        | —                      | 104                                | 2.6-3.1          | 400        | 200     |
| Naeaa    | 0.5                      | 2.8                    | 100                                | 2.5              | 12         | 10      |
| Naeaa    | 0.5                      | 1.2                    | 100                                | 2.5              | 55         | 20      |
| Naeaa    | 3                        | 3.05                   | 104                                | 2.5-3.0          | 40         | 35      |
| Naeaa    | 3                        | 3.1                    | 104                                | 2.5-3.0          | 10         | 10      |
| Naeaa    | 6                        | 3.1                    | 104                                | 2.5-3.1          | 25         | 25      |

The results of Table 3A are considered inconclusive, at best. It is the present inventor's opinion that the rather indifferent performance of the additive probably resulted from the low corrosion rates which existed even in the absence of additive.

From the results reported in Table 3B, it can be seen that the corrosion was indeed effectively reduced; and these results are seen to indicate the efficacy of the additive in reducing the corrosion of surfaces exposed to combustion gases in the cold-end of a boiler system.

#### EXAMPLE 4

In addition to analyzing the washings from the CERL probe for iron content, the total solids content of each sample was also determined to evaluate the fouling tendencies of the subject treatment. While it is expected that an additive treatment at the cold-end of a boiler system will cause some fouling, the additive is considered more effective as its fouling tendencies decrease.

The results of these tests are reported below in Tables 4A and 4B. In each of the preliminary tests, the results of which are reported in Table 4A, the probe was exposed to the combustion gases for a period of 0.5 hour; while in each of the confirming tests, the results of which are reported in Table 4B, the probe was exposed for a time period as indicated. The total solids are reported as parts of total solids per million parts of washing water at the probe surface temperatures indicated.

TABLE 4A

| Addi-<br>tive | Feed-<br>rate<br>(pph) | Steam Load<br>(pph $\times 10^3$ ) | % O <sub>2</sub> | Total Solids (ppm) |         |         |
|---------------|------------------------|------------------------------------|------------------|--------------------|---------|---------|
|               |                        |                                    |                  | 230° F.            | 250° F. | 300° F. |
| None          | —                      | 50                                 | 3.7              | 100                | 60      | 40      |
| Naeaa         | 3.4                    | 50                                 | 3.8              | 170                | 80      | 180     |
| Naeaa         | 1.2                    | 53                                 | 4.1              | 140                | 150     | 80      |

TABLE 4B

| Additive | Exposure Time (hours) | Feedrate (pph) | Steam Load (pph $\times 10^3$ ) | % O <sub>2</sub> | Total Solids |         |         |
|----------|-----------------------|----------------|---------------------------------|------------------|--------------|---------|---------|
|          |                       |                |                                 |                  | 230° F.      | 250° F. | 300° F. |
| None     | 0.5                   | —              | 100                             | 2.5              | 460          | 250     | 75      |
| None     | 3                     | —              | 104                             | 2.5-3.0          | 1800         | 1300    | 150     |
| None     | 6                     | —              | 104                             | 2.6-3.1          | 3000         | 2000    | 400     |
| Naeaa    | 0.5                   | 2.8            | 100                             | 2.5              | 360          | 270     | 180     |
| Naeaa    | 0.5                   | 1.2            | 100                             | 2.5              | 340          | 220     | 80      |
| Naeaa    | 3                     | 3.05           | 104                             | 2.5-3.0          | 1200         | 1000    | 850     |
| Naeaa    | 3                     | 3.1            | 104                             | 2.5-3.0          | 750          | 650     | 450     |
| Naeaa    | 6                     | 3.1            | 104                             | 2.5-3.1          | 2600         | 2400    | 1400    |

Based on the results reported above in Tables 4A and 4B, the rate of solids deposition on the surfaces when the additives is used is considered to be acceptable.

15

## EXAMPLE 5

In another series of tests, the CERL probe was exposed to the combustion gases for various periods of time, removed, and visually inspected. The results are 20 reported below in Table 5.

TABLE 5

| Additive | Exposure Time (hours) | Appearance of Probe                                                            |    |
|----------|-----------------------|--------------------------------------------------------------------------------|----|
|          |                       | 25                                                                             | 25 |
| None     | 0.5                   | Green coating on cold-end of probe.                                            |    |
| None     | 3                     | Heavy green coating on cold-end.                                               |    |
| None     | 6                     | Very heavy green coating on cold-end, which coating was difficult to wash off. |    |
| Naeaa    | 0.5                   | Clean, glossy.                                                                 |    |
| Naeaa    | 3                     | No apparent build-up. Slightly tacky.                                          |    |
|          |                       | Easily washed.                                                                 |    |
| Naeaa    | 6                     | Shiny. Soot on leading edge. Sticky at cold-end. Easily washed.                |    |

Additional assessments were made based on various tests conducted using a D-type boiler manufactured by Keeler. The boiler is rated at 26,000 pounds of steam per hour and is normally operated at 200 psig pressure.

Since the primary function of a cold-end additive is to eliminate or reduce corrosion caused by the condensation of sulfuric acid, techniques that measure corrosion were expected to yield adequate information about product performance. Accordingly, the well known method of quantifying the reduction in corrosion of the above-described air-cooled probe was used for determining efficacy as cold-end additives. Flue gas constituents were allowed to condense on the probe for 45 minutes. The probe was then immediately washed with doubly distilled water and analyzed for iron and sulfate. Corrosion was measured by analyzing the probe washings for water soluble iron, which is also a well known technique.

Since a cold-end additive should be capable of traveling along with the combustion gases and depositing on the downstream cold-end surfaces to be treated, the various additives tested were sprayed, using a standard

atomizing spray nozzle arrangement, into the combustion gases at a point of turbulence located upstream of the air cooled probe.

Immediately before base loading, the boiler was taken through a soot blowing cycle, and the burner tip was manually cleaned. The boiler was then based loaded for one hour. Fuel oil of precisely the same composition must be fired over a given period of time to ensure reproducibility of baseline data throughout the period. However, for critical testing, daily determination of baseline data is recommended.

The boiler was fired with number 6 grade fuel oil containing 1% sulfur (by weight). The oil was pre-heated to 170° F. and atomized with steam. Combustion air was at ambient temperature. Flue gas temperatures at the sampling point ranged from 440° F. to 480° F. The sulfuric acid dew point using either a Land dew point meter or a corrosion probe was typically 262° F. Using a Research Appliance Corporation sampling device, the concentration of SO<sub>3</sub> was determined to be about 7 parts per million parts of combustion gas (ppm, on volume basis). The oxygen content of the flue gas was kept at about 6%.

The materials tested were monoethanolamine, obtained from Fisher; 2-(ethylamino)ethanol, obtained from Fisher; 3-amino-1-propanol, obtained from Eastman; 2-amino-2-methyl-1-propanol, obtained from IMC; 2-dibutyl-aminoethanol, obtained from Eastman; 2-amino-2-ethyl-1,3-propanediol, obtained from Aldrich; 1-amino-2-propanol, obtained from Eastman; triethanolamine, obtained from Eastman; and diisopropanolamine, obtained from Dow.

The results of a first series of tests are reported below in Table 6, wherein a different test number indicates that tests were conducted on a different day.

The additive feedrates are reported as pound(s) of additive per pound of SO<sub>3</sub> generated (lb. Additive/lb. SO<sub>3</sub>), and the probe corrosion results are reported as % reduction in iron content of the probe washings for the indicated temperatures as compared to base condition corrosion. Negative results indicate a condition of increased corrosion of the probe as compared to base condition. The steam loads are reported as pounds per hour (pph).

TABLE 6

## CORROSION INHIBITION OBTAINED WITH A NUMBER OF ALKANOLAMINES

| Test | Additive                    | lb. of Additive/<br>lb. of SO <sub>3</sub> | Steam Load<br>(pph $\times 10^3$ ) | Mole of Additive/<br>bbl. of Oil Consumed | % Reduction in Fe vs.<br>Temperatures, °F. |     |     |     |
|------|-----------------------------|--------------------------------------------|------------------------------------|-------------------------------------------|--------------------------------------------|-----|-----|-----|
|      |                             |                                            |                                    |                                           | 205                                        | 215 | 225 | 235 |
| 1    | 2-(ethylamino)-ethanol      | 1.3                                        | 11-12                              | 1.0                                       | 95                                         | 93  | 95  | 92  |
|      | 3-amino-1-propanol          | 1.0                                        | 11-12                              | 1.0                                       | 97                                         | 95  | 96  | 93  |
|      | 2-amino-2-methyl-1-propanol | 1.3                                        | 11-12                              | 1.0                                       | 96                                         | 93  | 92  | 88  |
|      | 2-dibutyl-aminoethanol      | 2.4                                        | 11-12                              | 1.0                                       | 60                                         | 48  | 45  | 23  |
| 2    | 2-(ethylamino)-ethanol      | 0.6                                        | 11-13                              | 0.5                                       | 58                                         | 50  | 44  | 35  |
|      | 3-amino-1-propanol          | 0.4                                        | 11-13                              | 0.4                                       | 48                                         | 41  | 36  | 30  |
|      | 2-amino-2-methyl-1-propanol | 0.3                                        | 11-13                              | 0.3                                       | 6                                          | -15 | -33 | -49 |

TABLE 6-continued

## CORROSION INHIBITION OBTAINED WITH A NUMBER OF ALKANOLAMINES

| Test | Additive                        | lb. of Additive/       | Steam Load               | Mole of Additive/    | % Reduction in Fe vs. |     |     |     |
|------|---------------------------------|------------------------|--------------------------|----------------------|-----------------------|-----|-----|-----|
|      |                                 | lb. of SO <sub>3</sub> | (pph × 10 <sup>3</sup> ) | bbl. of Oil Consumed | 205                   | 215 | 225 | 235 |
| 3    | 2-amino-2-ethyl-1,3-propanediol | 0.6                    | 12.5-13.8                | 0.4                  | 67                    | 55  | 51  | 48  |
|      | 1-amino-2-propanol              | 0.4                    | 12.5-13.8                | 0.4                  | 35                    | 34  | 35  | 26  |
|      | diethanolamine                  | 0.6                    | 12.5-13.8                | 0.4                  | 62                    | 53  | 49  | 38  |

As can be seen from the results reported in Table 6, a variety of alkanolamines demonstrated cold-end additive efficacy.

The results of a second series of tests are reported below in Table 7, wherein a different test number indicates that tests were conducted on a different day. The additive feedrates are reported as mole per barrel of oil consumed (mole/bbl), and the corrosion results are reported as % reduction in iron content of the probe washings for the indicated temperatures. These test results are seen to demonstrate the ability of the alkanolamines tested to reduce cold-end corrosion.

ble alkanolamine such that said additive will travel along with said gases, as vapor and/or liquid droplets, from said zone of turbulence to said second zone and deposit on surfaces of said metal parts.

2. The method of claim 1, wherein an aqueous solution of the additive is added to the combustion gases.

3. The method of claim 1, wherein the alkanolamine is added in an amount of from about 0.1 to about 2.0 pound per pound of sulfur trioxide produced upon combustion of the fuel.

4. The method of claim 3, wherein the alkanolamine is added in an amount of from about 0.25 to about 1.0

TABLE 7

| Test | Additive                    | Steam Load<br>(pph × 10 <sup>3</sup> ) | Additive Feedrate<br>(mole/bbl) | % Reduction in (Fe) |         |         |           |
|------|-----------------------------|----------------------------------------|---------------------------------|---------------------|---------|---------|-----------|
|      |                             |                                        |                                 | 190° F.             | 200° F. | 230° F. | 250° F.   |
| 1    | N-aminoethyl ethanolamine   | 11-11.5                                | 0.88                            | 94                  | 65      | 42      | 27        |
| 2    | monoethanolamine            | 11.5                                   | 0.84                            | 85                  | 74      | 33      | 0         |
| 3    | 2-amino-2-methyl-1-propanol | 13.0                                   | 0.42                            | 58                  | 47      | 25      | Corrosive |
| 4    | monoethanolamine            | 13.0                                   | 0.46                            | 56                  | 52      | 38      | Corrosive |
| 5    | monoethanolamine            | 13.5-14                                | 0.12                            | 36                  | 40      | 42      | 0         |
|      | N-aminoethyl ethanolamine   | 13.5-14                                | 0.12                            | 39                  | 11      | 51      | 0         |
|      | triethanolamine             | 13.5-14                                | 0.13                            | 25                  | -24     | 18      | 0         |
|      | ethylamine                  | 13.5-14                                | 0.12                            | 0                   |         |         |           |
| 6    | monoethanolamine            | 13-14                                  | 0.39                            | 74                  | 48      | 50      | 0         |
| 7    | monoethanolamine            | 13-14                                  | 0.34                            | 83                  | 75      | 72      | 69        |
| 8    | monoethanolamine            | 13.5-14.8                              | 0.34                            |                     | 25      | 36      | Corrosive |
| 9    | diisopropanolamine          | 13.5-14.8                              | 0.36                            |                     | 23      |         | CORROSIVE |
| 10   | monoethanolamine            | 14.2-15.5                              | 0.31                            |                     | 46      | 36      | 31        |
|      | 2-ethylamino ethanol        | 14.2-15.5                              | 0.31                            |                     | 41      | 27      | 0         |
|      | N-aminoethyl ethanolamine   | 14.2-15.5                              | 0.33                            |                     | 79      | 78      | 73        |
|      | monoethanolamine            | 14.2-15.5                              | 0.31                            |                     | 46      | 36      | 31        |
| 11   | 2-dibutylaminoethanol       | 15-16                                  | 0.37                            |                     | 40      | 27      | Corrosive |
| 12   | 3-amino-1-propanol          | 13.5-14.5                              | 0.36                            |                     | 43      | 13      | 0         |
|      | 1-amino-2-propanol          | 15.5-16.5                              | 0.27                            |                     | 38      | 0       | CORROSIVE |

In test number 5 of Table 7 are reported the results of a run using ethylamine, a known SO<sub>x</sub> gas neutralizer in wet gas scrubbers. From these results, it can be seen that the ethylamine was unsuitable for the purpose of reducing corrosion, particularly as compared to various alkanolamines fed at the same rate to the flue gas.

In additional tests in which both ethylamine and N-aminoethyl ethanolamine were both fed to the combustion gas of a boiler at the rate of 0.87 mole/hour, the 50 ethylamine again proved to be very corrosive while the N-aminoethyl ethanolamine effectively reduced corrosion of the test probe. The ethylamine is, accordingly, seen to be unsuitable as a cold-end additive.

Having thus described the invention, what is claimed is:

1. A method of reducing the amount of sulfur trioxide condensation on, and therefore the amount of sulfuric acid corrosion of, metal parts at the cold-end of a combustion system in contact with combustion gases derived from the combustion of sulfur-containing fuel, which combustion gases flow along a path at the cold-end of the combustion system from a first zone of relative turbulence to a second zone at which the turbulence subsides, said method comprising:

adding to the combustion gases at the cold-end of the combustion system and at the zone of turbulence an effective amount for the purpose of an alkanolamine additive comprising an aliphatic, water-solu-

55 pound per pound of sulfur trioxide produced upon combustion of the fuel.

5. The method of claim 1, wherein the alkanolamine is added in droplet form to the combustion gases.

6. The method of claim 5, wherein the temperature of the combustion gases at the time of addition is from about 250° F. to about 675° F.

7. The method of claim 1, wherein the temperature of the combustion gases at the time of addition is from about 250° F. to about 675° F.

8. The method of claim 7, wherein the temperature of the combustion gases at the time of addition is from about 350° F. to about 650° F.

9. The method of claim 1, wherein the combustion system is a steam generating system, and wherein the fuel is sulfur-containing oil.

10. The method of claim 9, wherein the alkanolamine is added in droplet form to the combustion gases.

11. The method of claim 10, wherein the temperature of the combustion gases at the time of addition is from about 250° F. to about 675° F.

12. The method of claim 10, wherein an aqueous solution of the additive is added to the combustion gases.

13. The method of claim 12, wherein the additive is monoethanolamine.

\* \* \* \* \*